

## 1

2,955,960

MODIFICATION OF THE PROPERTIES OF  
SYNTHETIC FIBRES

John Woolley Batty, Albert Ewart Henshall, and Harold Sagar, Manchester, England, assignors to Imperial Chemical Industries Limited, London, England, a corporation of Great Britain

No Drawing. Filed Feb. 25, 1957, Ser. No. 641,827

Claims priority, application Great Britain Mar. 7, 1956

6 Claims. (Cl. 117—138.8)

This invention relates to modification of the properties of synthetic fibres and the modified synthetic fibres so obtained.

Certain synthetic fibres, especially those prepared from polyesters or polyamides or from cellulose acetate, show a tendency to accumulate a charge of static electricity during manufacturing operations, such as carding, spinning or weaving. It is with such synthetic fibres, that this invention is concerned; we have found that by a simple treatment, this undesirable tendency can be very considerably reduced.

Thus according to the present invention we provide a process for modifying the properties of synthetic fibres in particular for reducing the tendency thereof to accumulate a charge of static electricity, which comprises treating the fibres with a condensation product of from one to three molecular proportions of a fatty acid with one molecular proportion of glycerine previously condensed with from 3—40 molecular proportions of ethylene oxide. Fatty acids for use in the manufacture of the condensation products used in the process of this invention include oleic, stearic and lauric acids.

The treatment of the synthetic fibres according to the process of this invention may be achieved by any convenient means, for example by spraying the fibres with an aqueous or organic liquid solution of the condensation product or by immersing or padding the fibres in such a solution. The treatment may be at normal or elevated temperature. The impregnated fibres after removal from the treatment bath may be dried at any suitable temperature, from room temperature up to about 150° C.

The amount of condensation product deposited on the fibre may be from .05 to 1% by weight of the fibre.

The synthetic fibres to be treated may be in any form, such as yarn or fabric.

The condensation products used in the process of this invention are preferably liquid. It is frequently found that anti-static processing acids hitherto employed, being of a solid or waxy nature, tend to be scraped off the fibre, or to be deposited on the processing machinery, or on healds or guides so that an erratic performance is obtained which leads to subsequent spinning and weaving irregularities. These disadvantages are obviated or minimised when liquid agents are used, since the agent is present in the form of a uniform film on the fibre.

The invention is illustrated but not limited by the following examples in which parts and percentages are by weight.

The anti-static effect produced by the treatments in the examples was determined by measurement of the charge developed on rubbing the treated fabric against a Botany wool serge surface in the manner described in American Dyestuff Reporter, volume 40, No. 5, page 164, the charge being expressed in terms of current (measured in arbitrary units) in the peak voltmeter circuit. In all cases the fabrics were dried and conditioned prior to testing.

## 2

## EXAMPLE 1

A polyethylene terephthalate staple fibre fabric was padded in an aqueous solution of a condensation product of one molecular proportion of lauric acid with one molecular proportion of glycerine previously condensed with 6 molecular proportions of ethylene oxide.

The mangle expression and solution strength were adjusted so that 0.2% of the agent was applied to the fibre. The results are given in Table I.

## EXAMPLE 2

Example 1 was repeated, using a condensation product of one molecular proportion of lauric acid with one molecular proportion of glycerine previously condensed with 24 molecular proportions of ethylene oxide.

## EXAMPLE 3

Example 1 was repeated, using a nylon fancy weave fabric.

## EXAMPLE 4

Example 2 was repeated, using a nylon fancy weave fabric.

## EXAMPLE 5

Example 1 was repeated, using a condensation product of three molecular proportions of lauric acid with one molecular proportion of glycerine previously condensed with 24 molecular proportions of ethylene oxide.

## EXAMPLE 6

0.1% of a condensation product of one molecular proportion of lauric acid with one molecular proportion of glycerine previously condensed with 24 molecular proportions of ethylene oxide was applied to a cellulose acetate satin fabric by padding. The result is given in Table I.

Table I

## STATIC CHARGE MEASUREMENTS

[Relative Humidity: 65% at 21° C.]

| 45 | Treatment as in<br>Example     | Fabric                         | Static Charge                  |                                             |
|----|--------------------------------|--------------------------------|--------------------------------|---------------------------------------------|
|    |                                |                                | Maximum<br>Charge<br>developed | Time to fall<br>to half value<br>in seconds |
| 1  |                                | Polyethylene<br>terephthalate. | 280                            | 1                                           |
| 50 | 2                              | do                             | 120                            | 1                                           |
| 3. | Nylon                          |                                | 12                             | 1                                           |
| 4. | do                             |                                | 8                              | 1                                           |
| 5. | Polyethylene<br>terephthalate. |                                | 128                            | 1                                           |
| 6. | Cellulose ace-<br>tate.        |                                | 10                             | 1                                           |
| 55 | Untreated fabric               | Polyethylene<br>terephthalate. | 2,300                          | 32                                          |
|    | Untreated fabric               | Nylon                          | 1,400                          | 12                                          |
|    | Untreated fabric               | Cellulose ace-<br>tate.        | 310                            | 28                                          |

## EXAMPLE 7

0.15% of a condensation product of one molecular proportion of lauric acid with one molecular proportion of glycerine previously condensed with 22 molecular proportions of ethylene oxide was applied to nylon staple fibre (1½ inch, 1½ denier) from aqueous solution by spraying. After conditioning for 48 hours at 65% relative humidity at 21° C., the staple fibre was processed on a conventional revolving flat card followed by passage through a draw frame of the type used for processing cotton and the resulting slivers spun to yarn (60's cotton count) on a high draft ring frame.

Regular yarns of good strength were produced.

## 3

## EXAMPLE 8

Example 1 was repeated using a condensation product of stearic acid with one molecular proportion of glycerine previously condensed with 12 molecular proportions of ethylene oxide. The results are given in Table 2.

## EXAMPLE 9

Example 8 was repeated using a nylon staple fibre fabric.

## EXAMPLE 10

Example 1 was repeated using a condensation product of oleic acid with one molecular proportion of glycerine previously condensed with 18 molecular proportions of ethylene oxide.

## EXAMPLE 11

Example 10 was repeated using a nylon staple fibre fabric.

## EXAMPLE 12

Example 1 was repeated using a condensation product of stearic acid with one molecular proportion of glycerine previously condensed with 13 molecular proportions of ethylene oxide.

## EXAMPLE 13

Example 12 was repeated, using a nylon staple fibre fabric.

Table 2

STATIC CHARGE MEASUREMENTS  
[Relative Humidity: 65% at 21° C.]

| Treatment as in Example | Fabric                      | Static Charge            |                                       |
|-------------------------|-----------------------------|--------------------------|---------------------------------------|
|                         |                             | Maximum Charge developed | Time to fall to half value in seconds |
| 8                       | Polyethylene terephthalate. | 300                      | 1.                                    |
| 9                       | Nylon                       | 340                      | 1.                                    |
| 10                      | Polyethylene terephthalate. | 305                      | 1.                                    |
| 11                      | Nylon                       | 355                      | 1.                                    |
| 12                      | Polyethylene terephthalate. | 330                      | 1.                                    |
| 13                      | Nylon                       | 240                      | 1.                                    |
| 14                      | Polyethylene terephthalate. | 295                      | 1.                                    |
| 15                      | Nylon                       | 210                      | 1.                                    |
| 16                      | Polyethylene terephthalate. | 260                      | 1.                                    |
| 17                      | Nylon                       | 180                      | 1.                                    |
| Untreated fabric        | Polyethylene terephthalate. | 4,000                    | greater than 180.                     |
| Untreated fabric        | Nylon                       | 2,050                    | 32.                                   |

## EXAMPLE 14

Example 1 was repeated using a condensation product of stearic acid with one molecular proportion of glycerine

55

## 4

previously condensed with 24 molecular proportions of ethylene oxide.

## EXAMPLE 15

Example 14 was repeated using a nylon staple fibre fabric.

## EXAMPLE 16

Example 1 was repeated using a condensation product of oleic acid with one molecular proportion of glycerine previously condensed with 36 molecular proportions of ethylene oxide.

## EXAMPLE 17

Example 16 was repeated using a nylon staple fibre fabric.

15 What we claim is:

1. A process for minimizing the tendency to accumulate static electricity on synthetic fibers normally subject to such accumulation which comprises treating said fibers with a liquid, water-soluble condensation product of from one to three molecular proportions of a higher saturated fatty acid with one molecular proportion of glycerine previously condensed in the absence of water with from 3-40 molecular proportions of ethylene oxide.

2. The process of claim 1 wherein said fibers comprise a polymer selected from the group consisting of polyesters and polyamides.

3. The process of claim 1 wherein said fibers comprise cellulose acetate.

4. The process of claim 1 wherein said higher saturated fatty acid contains from 12 to 18 carbon atoms.

5. Process for modifying the properties of synthetic fibers as claimed in claim 1 wherein the amount of condensation product deposited on the fiber is from .05 to 1% by weight of the fiber.

35 6. A process for minimizing the tendency to accumulate static electricity on polyethylene terephthalate fibers normally subject to such accumulation which comprises treating said fibers with a liquid, water-soluble condensation product of from one to three molecular proportions of a higher saturated fatty acid with one molecular proportion of glycerine previously condensed in the absence of water with from 3-40 molecular proportions of ethylene oxide, the amount of condensation product deposited on the fiber being from .05 to 1% by weight of the fiber.

## References Cited in the file of this patent

## UNITED STATES PATENTS

50 2,418,752 Brown Apr. 8, 1947  
2,450,079 Brown Sept. 28, 1948  
2,461,043 Eisen Feb. 8, 1949

## FOREIGN PATENTS

380,431 Great Britain Sept. 12, 1932